

Nov. 15, 1960

F. D. DE VANNEY

2,960,396

PELLETIZATION OF IRON ORE CONCENTRATES

Filed Dec. 23, 1957



Fig. 1



Fig. 2

Inventor

Fred D. De Vanney,

By Pierce, Schefler & Parker

his Attorneys

2,960,396

**PELLETIZATION OF IRON ORE CONCENTRATES**

 Fred D. De Vaney, Duluth, Minn., assignor to P-M  
Associates, Cleveland, Ohio, a copartnership

Filed Dec. 23, 1957, Ser. No. 704,609

6 Claims. (Cl. 75—3)

This invention relates to the art of preparing finely divided iron ore materials, e.g., concentrates, in a form suitable for subsequent use in a blast furnace or open hearth furnace, and is particularly concerned with the pelletization (including both (a) forming into small balls or pellets and (b) indurating the pellets so formed) of such finely divided iron ore materials as comprise a substantial proportion of a relatively non-magnetic oxidic compound of iron including the minerals hematite, specularite (specular hematite), limonite and siderite. The invention will, in the following, be discussed with more specific reference to pelletizing specularite concentrates.

The pelletization of finely divided specularite is peculiarly troublesome because of the nature of its particles. Specularite per se occurs in the form of well-developed platey crystals of hexagonal system, which crystals may be accompanied by a relatively small amount of particles finer than 1 micron (so-called "colloidal" fraction). Specularite is relatively difficult to grind. In any of the systems commonly employed for concentrating specularite which has been ground to size of liberation—e.g., flotation, or gravity separation using Humphrey spirals—it is customary if not essential preliminarily to remove from the ground material all particles finer than 10 microns (the conventional preliminary "de-sliming" treatment) in order to expedite the particular concentrating procedure which is to follow. The de-slimed concentrate, because of its distinctly platey nature and because of the absence of very fine particles, is practically impossible to ball up in a conventional balling apparatus (inclined rotary drum, or balling cone, or "pan"-type pelletizer), and any pellets so formed have exceedingly poor mechanical strength both in the "green" (non-heat-treated) or in the "fired" (heat-treated) stage.

In evaluating the ballability of an iron ore concentrate, the amount of material passing a minus 325 mesh screen has conventionally been held to be the criterion in describing the structure of a concentrate which balls well. This is a very rough measurement. Actually, it has been found that the balling characteristics depend on the proportion of the material which is in minus 1 micron, or "sub-micron," range. For example, in the case of an iron ore concentrate which is all minus 325 mesh and contains a substantial amount of material finer than 10 microns (which material, "as is," balls very well and produces a pellet having good green strength), if one de-slimes this ground product—removing from it substantially all of its content of minus 10 micron particles—the de-slimed material would not ball at all or would ball so poorly as to be unacceptable. Conversely, a ground product containing sizes as coarse as 10 mesh and only 50% finer than minus 325 mesh, but containing about 10% of material finer than 10 microns, balls readily and the pellets usually have good green strength. The fact that no problem arises in balling concentrates from earthy hematites is explainable on the basis of substantial absence therefrom of platey crystals and of the presence

therein of a substantial content of minus 10 micron particles.

The particle size distribution of a specularite concentrate obtained, from a predominantly non-magnetic lean ore (found in the Wabush Lake area, Labrador), by crushing and grinding to the particle size of liberation, de-sliming and gravity concentration on Humphrey spirals may be illustrated in column "A" of Table I following. For comparison, in columns "B" and "C" are given 10 screen analyses of two different magnetite concentrates.

TABLE I

|    | Mesh  | A<br>Specularite Conc. | B<br>Magnetite Conc. | C<br>Magnetite Conc. |
|----|-------|------------------------|----------------------|----------------------|
| 15 | +14   | 0.6                    |                      |                      |
|    | -20   | 1.6                    |                      |                      |
|    | +28   | 3.4                    |                      |                      |
| 20 | +35   | 7.5                    |                      |                      |
|    | -48   | 13.4                   |                      |                      |
|    | +65   | 22.5                   | 1.0                  | 0.18                 |
|    | +100  | 16.0                   | 2.5                  | 0.45                 |
|    | +150  | 13.2                   | 3.9                  | 1.73                 |
|    | +200  | 8.4                    | 7.0                  | 3.78                 |
| 25 | +325  | 7.4                    | 20.6                 | 12.92                |
|    | -325  | 6.0                    | 65.0                 | 80.94                |
|    | Total | 100.0                  | 100.0                | 100.00               |

In connection with the foregoing Table I, it may be noted that the data given in column C are illustrative of a magnetite concentrate commercially produced by Erie Mining Company, at its commercial beneficiation plant near Aurora, Minnesota, U.S.A., from a taconite whose iron content consists essentially of fine magnetite, the beneficiation procedure employed including the steps of crushing, grinding and magnetically separating the magnetite particles as a concentrate. The concentration is then agglomerated by filtering, mixing the filter cake with finely divided anthracite (about 10 lbs. per long ton, dry weight, of concentrate) and bentonite (about 12 lbs. per long ton, dry weight, of concentrate), balling the mixture in a balling drum, and indurating the small balls or pellets in a shaft-type indurating furnace at a maximum heat-treating temperature of 2350° F. or above. In the commercial operation aforesaid, certain practical criteria have been set up for evaluating the mechanical strength or ruggedness of the balls or pellets, viz.

Drop test No. At least 6.  
50 Compression test, green pellets At least 8 lbs.  
Compression test, pellets dried at  
250° F. 35 lbs. and above.  
Compression test, pellets fired at  
2350° F. 1,000 lbs. and above.

55 A "drop test" number of "6" means that the average green pellet can be dropped six times from a height of 18 inches before it breaks. This figure gives an indication of the resistance of the green pellet to the breakage of pellets in passing from the balling drum to the first conveyor, and from one conveyor to another, and from the last conveyor onto the furnace loader and from the loader onto the top of the charge column in the furnace: in a real sense, it is a measure of the resiliency of the green pellet.

60 The "compression test" measures the strength of the pellet, in the number of pounds required to break the pellet. It has been found that if a pellet has a compression strength less than 8 lbs. the loading of material on 70 the pellet in the upper part of the furnace shaft will break the pellet.

In attempting similarly to agglomerate the specularite

concentrate referred to in column A of Table I, using 15 lbs. of bentonite per long ton, dry weight, of concentrate, the strength data for the pellets were:

Drop test No. 1.5  
Compression test, green pellets lbs. 2  
Compression test, pellets dried at 250° F. lbs. 8  
Compression test, pellets fired at 2350° F. lbs. 400

The green pellets were of very inferior quality, and they could neither be handled by conveyors nor fired on any type of grate sintering machine or shaft-type indurating furnace to give a satisfactory result.

It heretofore had been thought that the above-described disadvantages in pelletizing specularite concentrates arose from mere particle size and particle size distribution, and that the way to improve the ballability of the specular hematite concentrate was to subject it—or, a part of it—to finer grinding whereby to increase the proportion of finer sizes of particles in the material to be balled. However, it was found that finer grinding did not solve the problem, due undoubtedly to the fact that the more finely ground specularite, while, it is true, being of smaller particle size, nevertheless was grainy (well crystallized) and provided little or no plasticity to the concentrate mixture to be pelletized; while the mixture containing the more finely ground material showed some improvement as to ballability, the resulting pellets were extremely fragile (would not withstand necessary handling in the "green" state) and broke down badly on firing. This unsatisfactory situation could, to some extent, be corrected by homogeneously dispersing through the specularite concentrates—e.g., concentrates a part or all of which had been subjected to fine grinding, as aforesaid—a relatively very large amount (of the order of 5% by weight, more or less) of bentonite. However, the inclusion in the pelletized product of such a large amount of "foreign" material of this sort was both economically and technologically unfeasible, because of the added cost of the large amount of bentonite and because the product would be "adulterated" with so large a proportion of non-ferrous material not desirable for burdening the blast furnace.

It has now been found that the ballability of a specularite concentrate can be greatly improved, and that the mechanical strength of pellets consisting largely of specularite particles can be greatly increased, by homogeneously dispersing through the specularite concentrate—prior to balling—a substantial proportion of a concentrate of finely divided magnetite particles, either natural magnetite or the "artificial magnetite" produced by subjecting an iron ore the content of oxidic compound of iron of which is essentially non-magnetic iron oxide, e.g., hematite, limonite, or siderite, to reductive roasting under conditions to convert the iron oxides to  $Fe_3O_4$ . The added magnetite tends to give the balls a structure which cannot be duplicated in a ball of specularite only. The magnetite particles are largely isometric (not platy), and their inclusion in the specularite materially improves the ballability of the same, and materially adds to the green strength of the pellets and to their fired strength as well. All of the so-called "colloidal" material (i.e., material having a particle size less than 1 micron diameter) naturally occurring in the raw material is retained in the magnetite concentrate, to provide in the specularite-magnetite mixture the plasticity necessary for good balling and for good green strength and fired strength of the pellets.

In applying this discovery to the pelletization of a specular hematite concentrate, the amount of added magnetite, with respect to a unit amount of the specularite particles, may be adjusted within relatively wide limits depending upon the fineness of grind of the magnetite concentrate including particularly the relative content therein of very fine particles—minus 200 mesh plus 325 mesh, minus 325 mesh, and "sub-micron" particles—for enhancing the plasticity and promoting the balling of

the composite concentrate. In this connection, it frequently will be found desirable deliberately to over-grind the magnetite concentrate portion—substantially beyond the normal size of liberation of the magnetite—in order to have available a higher proportion of the finest particles.

Thus, in a situation where there is available, for the above purpose, a relatively large amount of magnetite concentrate, e.g., 75 parts of magnetite concentrate (the normal size of liberation of which is minus 48 mesh) and 25 parts of specular hematite concentrate, the magnetite will be ground to all minus 65 mesh in order to improve it as a binder. Where about as much magnetite is available as is the amount of specularite to be balled, it is desirable to grind the magnetite to essentially all finer than 100 mesh. Where the ratio of available magnetite to specularite is of the order of 35:65, the magnetite should be ground much finer, i.e., to minus 200 mesh. As an extreme example, where the ratio of available magnetite concentrate to specularite concentrate is only 15:85, it is necessary to grind the magnetite to all minus 325 mesh in order to provide the necessary plasticity and bonding of the particles of the composite.

As was suggested above, where a concentrate of natural magnetite is not available the same may be substituted by a concentrate of an "artificial" magnetite produced by reductively roasting a non-magnetic iron ore (e.g., a portion of the specular hematite ore, or an equivalent amount of an earthy hematite ore, or limonite or siderite ore) to prepare a concentrate therefrom after suitably fine-grinding, and admix such "artificial" magnetite concentrate with the specularite concentrate.

To illustrate, the so-called Jasper ores of Michigan, in which hematite ores specularite is frequently a major constituent, may be used as an example. Michigan Jasper ores are frequently concentrated by a flotation process in which, after the crude ore has been ground to liberation size (approximately minus 65 mesh), the ore is pulped, de-slimed, and the hematite recovered by flotation. It has been found virtually impossible to ball this flotation concentrate per se, and the expensive step of further grinding the material—to promote ballability—does not completely solve the problem, even with such further grinding and with the employment of much bentonite in the mix the characteristics of the resulting pellets, both as regards green strength and as regards fired strength, are so poor as to make these measures only partially effective.

However, by reductively roasting a substantial portion (e.g. from 15% to 50% or more) of the Jasper ore or its concentrate, over-grinding the resulting "artificial" magnetite, recovering a magnetite concentrate therefrom and adding the latter to the Jasper concentrate, the resulting composite concentrate has been found to have good balling characteristics and to yield pellets having good green strength (and, as well, good "fired" strength).

As will be appreciated from the foregoing, in lieu of reductively roasting the Jasper ore, whereby to obtain a material from which a magnetite "binder" may be recovered, one may reductively roast an earthy hematite and from the roasted material magnetically derive a magnetite concentrate suitable for admixture with the Jasper non-magnetic concentrate. Or, where an ore material containing natural magnetite is available, the same may be finely ground and magnetically concentrated to yield the necessary binder for the Jasper concentrate.

Where reductive roasting is restored to, the same may be carried out according to known technique. For example, the procedures disclosed in U.S. Patents Nos. 2,528,552, 2,528,553 and 2,670,946 may be followed for this purpose. As an alternative, the non-magnetic iron ore from which the "artificial" magnetite is to be prepared may be worked up by crushing the ore to suitable fine size and subjecting the crushed material to fluo-

solids reductive roasting, followed by further fine grinding, if necessary, and magnetic concentration.

It should be noted that, whatever the mode of reductive roasting selected, the roasted product is much easier to fine-grind than is the non-roasted material.

The magnetite component of the mixture of non-magnetic and magnetic iron ore materials may, as stated previously, be formed from a portion of the non-magnetic iron ore material by reductively roasting said portion, grinding the reduced material to very fine particle size, and magnetically separating the magnetite. In carrying out this procedure in the case of a boggy, wet or high-moisture, low-grade, ore material it may be found unfeasible or impossible to roast the material in its natural state, or to screen the raw material and thereafter roast the same by conventional methods. In such event, a portion of the high-moisture ore material can be balled up, in any known type of balling device such as a balling drum or balling cone, whereby to form the material into small pellets, and the balled material subjected to a reductive roast under conditions to convert the content of non-magnetic oxidic compound of iron to  $Fe_3O_4$ . In case these pellets are too fragile to be reductively roasted in a shaft-type furnace, they may be reductively roasted in a shallow bed (so as not to impose crushing loads on the feeble pellets) as on a horizontal traveling grate-type of furnace.

The above described concept of improving the ballability of iron ore concentrates consisting essentially, or largely, of specularite particles can be applied to other specularite concentrates than those obtained by flotation concentration; thus, they can be applied with equal effectiveness to a specularite concentrate obtained by a fine particle gravity-type concentration procedure such as the use of Humphrey's spirals.

#### Example 1

As an example of the balling phase of the invention, 70 parts of a specular hematite concentrate, having the size analysis given, under "specular hematite conc.", in Table I hereof, were admixed with 30 parts of a magnetite concentrate, having the size analysis given in column "C" of Table I. The specularite concentrate had a moisture content of 6.0%, while the magnetite concentrate had a moisture content of about 9.5%. To the mixture there were added, in pounds per long ton of mixture, dry weight, bentonite 10-20 and soda ash (dispersing agent) 1.0-1.5, together with an amount of finely divided solid carbonaceous fuel (coal, or coke) appropriate for the ensuing induration process. In the case of shaft furnace induration about 20 lbs./l.t. of finely divided fuel were used, whereas in the case of induration on a traveling grate type of apparatus 40-60 lbs./l.t. of fuel were called for. The amount of soda ash employed was dependent upon the pH of the mill water used.

The above components were homogeneously admixed, and the mixture was balled up in an inclined rotary balling drum, under conditions to "work" the mixture well for development of optimum plasticity. The mixture balled well, and the resulting pellets had ample green strength for transportation to the ensuing induration operation without damage.

Comparative strength data for these pellets averaged:

|                                              |        |
|----------------------------------------------|--------|
| Drop test No. _____                          | 6.1    |
| Compression test, green _____ pounds         | 10.2   |
| Compression test, dried at 250° F. _____ do  | 36.0   |
| Compression test, fired at 2450° F. _____ do | 1250.0 |

The following further specific example is illustrative of the improvements in ballability and in green strength and fired strength resulting from the practice of the above-stated concept.

#### Example 2

The starting material was a lean iron ore from the 75 drum to indurating furnace without breakage or distortion.

Wabush deposit, central Labrador, analyzing 37.3% Fe, the iron content of the ore occurring essentially in the forms of (a) specularite and (b) magnetite, in the approximate ratio of 7 parts specularite to 3 parts of magnetite, with a relatively small content of limonite.

The ore was crushed, and dry ground to approximately all minus 35 mesh in an Areofall mill, pulped with water, and concentrated magnetically to obtain two intermediate products, viz. (a) a non-magnetic portion containing essentially all of the specularite, and (b) a magnetic portion containing essentially all of the magnetite.

The non-magnetic portion represented 82.6% by weight of the total, and assayed 32.61% Fe and 48.99% Si, together with a small percentage of a non-magnetic tailing from a concurrent concentration of a magnetic portion of the total ore. This non-magnetic portion was deslimed and then concentrated by banks of Humphreys spirals in series. The resulting spirals concentrate represented 31.84% by weight of the total crude and had an analysis of 63.64% Fe and 4.89% Si. The sizing analysis of this product is given (under "specularite conc.") in Table I above.

Balling tests on the above non-magnetic concentrate showed that it was commercially impossible to ball it per se in any known type of balling equipment (inclined rotary balling drum, balling cone, or pan-type pelletizer); also, that what balls were rolled up were too fragile to be indurated in any known type of induration equipment (shaft furnace, up-draft or down-draft horizontal grate furnace, or combination grate-and-kiln).

The minus 35 mesh magnetic portion contained 62.03% Fe and 10.02% Si and represented about 31% by weight of the recovered iron (the specularite representing the remaining 69%): it was of a grade sufficiently high to be marketable. However, in order to obtain sufficient fines to permit balling a mixture of this concentrate and the above described specularite concentrate, the magnetite concentrate was further ground, in a ball mill, to minus 100 mesh and re-concentrated magnetically. The size analysis of this final magnetite concentrate is given in column "B" of Table I above. It is to be noted that this magnetic concentrate had been ground to a size materially finer than that necessary for liberation (i.e., finer than that necessary to produce a good grade of marketable concentrate) or for pelletizing it (if pelletized alone), this over-grinding being done purely to provide sufficient fines—including especially particles less than 10 microns in diameter—to promote the necessary binding functions with respect to the concurrently produced granular hematite concentrate described above.

The relative dry weights of the solids of the two concentrates were:

31.23% magnetite conc., and  
55 68.77% non-magnetic spirals conc.

After filtering, the two concentrates were admixed, and to the mixture there were added 12 lbs./long ton of bentonite and 1.5 lbs./long ton of soda ash (as disperser for the bentonite), together with 25 lbs./l.t. of finely divided anthracite coal. These components were very thoroughly mixed together (by the aid of a mixer-muller) until the mixture was homogeneous: it had an average moisture content of 8.5%.

The mixture was then balled in an inclined rotary balling drum, 3 ft. diameter by 8 ft. long, such as that described and claimed in my U.S. patent application Serial No. 211,290, filed February 16, 1951, now Patent No. 2,831,210, granted April 22, 1958. The mixture balled very well, forming pellets varying in diameter between 1.5 inches and one-fourth inch. These pellets, because of their content of finely ground magnetite in association with the small amount of bentonite, were of ample green strength to undergo transportation from

tion. The pellets were fed onto the top of a column of similar pellets in a generally cylindrical vertical shaft-type indurating furnace, 30 inches diameter, embodying the features of the furnace described in my U.S. patent application Serial No. 590,358, filed June 11, 1956, now Patent No. 2,816,016, granted December 10, 1957, at the approximate rate of 1800 lbs., dry weight, per hour. The temperature of the heating gas flowing from the combustion chambers was held at approximately 2400° F., and atmospheric air was introduced at the following rates:

|                            | C.f.m. |
|----------------------------|--------|
| At the bottom of the shaft | 225    |
| Into combustion chambers   | 105    |

The zone of maximum temperature was approximately 2450° F., and the temperature was substantially uniform (in the pellets column) from a horizon about one foot down from the stockline to the inlets from the combustion chambers, a vertical distance of about 6 feet: below the inlets, the temperature of the pellets column sloped downwardly through the cooling section of the furnace to an exit temperature of approximately 350° F. The spent gases exited from the stockline at about 180° F.

For maintaining the above combustion chambers temperature about 2.5 gals. of fuel oil, per long ton of finished product, were burned in the chambers, this amount of fuel oil together with the 25 lbs./l.t. of coal giving a total B.t.u. consumption of 612,500 per long ton of finished product. The oxidation of the magnetite content of the pellets contributed approximately 105,000 B.t.u.'s per long ton of finished product.

Average comparative strength data for these pellets did not differ significantly from those given in Example 1 above.

The finished product, when subjected to the A.S.T.M. standard coke tumble test, gave a hardness number of 84.0 using a 10 mesh screen as the index figure.

The data of the above example sharply distinguish from those obtaining in the case of the pelletization of an all-hematite concentrate relying wholly on "imported" heat. In the latter situation, it is necessary—in order to indurate to a hardness acceptable for shipment of the product to the lower lake ports—to push the maximum temperature to 2600–2700° F. in order to obtain the slag bond which is all that one can rely on in such an operation. This difference is critical, because the temperature level 2600–2700° F. is at the edge of the range where substantial actual melting occurs, and hence satisfactory commercial operation is very difficult if not impossible to accomplish. By resorting to the novel measures set forth in the above specific example, in which the maximum temperature was 2450° F., one can operate at a temperature safely below the fusing temperature of the hematite-silica concentrate, and hence enjoy uninterrupted operation of the indurating process with production of "fired" pellets which are essentially discrete.

It has been found, further, that the induration of pellets comprising non-magnetic oxidic compounds of iron—e.g. concentrates of earthy hematite, concentrates of oxidized (non-magnetic) taconite, as well as the above-described concentrates of Jasper ores and similar ores consisting largely of specular hematite—can be very materially improved, and that fired pellets of better characteristics can be produced, by the inclusion in such pellets, in homogeneous admixture with the non-magnetic particles, of a substantial proportion of natural or "artificial" magnetite along with whatever other additives may be included in the mixture. The expression "other additives" is meant to include, but not to be limited to, a conventional "binding" agent, e.g., starch, bentonite, waste sulfite liquor product or the like, and also finely divided solid carbonaceous fuel.

The homogeneous incorporation of finely divided magnetite in the mixture to be pelletized not only very materially improves the ballability of the non-magnetic (e.g. specular hematite or earthy hematite) particles, as above described, and materially increases the green strength of the resulting pellets, but also promotes better induration of the particles and a substantial improvement in their "fired" strength.

10 The induration of iron ore pellets whose content of oxidic compound of iron consists almost wholly of a non-magnetic oxide of iron has long been known to be much more difficult than indurating pellets of magnetite. It heretofore had been proposed to effect the induration of such non-magnetic ore pellets by including within 15 them a relatively very large amount of solid carbonaceous fuel whereby—through the medium of the heat of combustion of the fuel throughout the structure of the pellet—to bring all parts of the pellet to the necessary hardening temperature.

20 I have found that substitution of finely divided magnetite for a part of the solid carbonaceous fuel content of these pellets produces a new and different result, arising from two phenomena. In the first place, the temperature level at which oxidation of magnetite to hematite is active is materially higher than is the ignition temperature of solid carbonaceous fuel, which circumstance brings it about that the heat of the magnetite oxidation is developed in the pellets column or bed at a level somewhat farther down from the top of the column or bed

25 than that at which the fuel begins to burn. Added coal (or, coke) dust, because of its relatively low ignition, tends to burn in the pellets in the upper few inches of the bed. Although the heat so liberated is beneficial (in driving off moisture and in pre-heating the pellets), it does not contribute desirably to the maximum temperature necessary or desirable for thorough induration of the pellets. The finely divided magnetite, on the other hand, begins to oxidize with fair rapidity at about 800° F. with desirably rapid release of heat; that is to say, its

30 heat is provided at a level (in the bed) where one wants to develop the "peak" temperature. This circumstance is advantageous in most cases, because it normally results in less loss of heat to the exiting gases and it tends to promote a more thorough heating of the pellets. In 35 the second place, the inclusion of finely divided magnetite throughout the structure of the pellet brings it about that during the ensuing induration the magnetite undergoes grain growth, so that there is developed within the pellet a network of binder which materially enhances the ruggedness and hardness of the fired pellets. Addition of

40 finely subdivided magnetite to the hematite not only contributes heat of oxidation where it is most needed but, more importantly, it provides about the coarser hematite particles a layer or film of magnetite which, by reason of the high-temperature oxidation and resulting grain 45 growth, enmeshes the hematite particles in a crystalline complex formed in situ about the hematite particles resulting in a very strong bonding of all particles together within the pellet. For both of these reasons, magnetite

50 within the pellets functions in a different way than coal and brings about a result distinct from that realizable through the use of solid carbonaceous fuel only, no matter how large a proportion of the latter is relied upon. In this connection, it should be noted that the grain growth function of the magnetite is particularly important.

55 Further improvement in the pelletization is realized by using the magnetite in very finely divided form—generally, more finely divided than would be necessary for liberation—whereby a unit amount by weight of the magnetite may more extensively and intimately be associated with the non-magnetic iron ore particles of the pellet. This improvement is not duplicated by omitting the magnetite and merely more finely grinding the non-magnetic iron ore particles to be pelletized.

While the above advantages are particularly important when the induration is being carried out in a vertical shaft-type indurating furnace, they apply also in grate furnace indurating furnace procedure because here, also, the heat line moves down (or, up) through a bed of the pellets. The heat of oxidation of magnetite—associated with the non-magnetic iron ore particles—contributes to the induration of the pellets in horizontal traveling grate furnaces of the downdraft and updraft types and also in kiln induration.

Moreover, to the extent that magnetite rather than coal contributes the within-the-pellets heat, the surrounding gases are maintained more highly oxidizing.

Fired pellets of the hematite-magnetite mixture result in less breakage and create less flue dust and the pellets are more dense than are fired pellets of hematite in the induration of which solid carbonaceous fuel was relied upon as the sole source of within-the-pellets heat, and there is less "dilution" by reason of "foreign matter" (i.e. ash).

The operating technique for indurating pellets of hematite-magnetite mixture is generally the same as that practiced in indurating all-magnetite pellets. The use of some coal (or other finely divided solid carbonaceous fuel) within the pellets is unavoidable in order to supplement the heat derived from oxidation of the magnetite content of the composite. The temperature of the oxidizing heating gas (e.g., of the highly heated air) used is to be regulated with respect to the heat to be derived from the magnetite plus the coal so that the pellets are thoroughly heated, throughout, at a temperature close to but safely short of that temperature at which the pellets would fuse together.

While the induration of pellets composed of hematite and finely divided magnetite is, herein, described with particular reference to use of a shaft furnace, it is to be understood that the inclusion of magnetite is of advantage when indurating in an updraft or downdraft horizontal traveling grate furnace or in a rotary kiln-type of furnace: the same phenomena which give strength as regards shaft furnace operation generally apply. This concept would, also, be helpful in indurating by a combination of horizontal grate and kiln.

As was intimated above, the amount of solid carbonaceous fuel used is to be varied to complement the particular amount of magnetite present in the pellets, and also with regard to the type of indurating procedure to be followed. Thus, if the mixture were 85% hematite and only 15% finely divided magnetite, the coal content would have to be of the order of 40 lbs./l.t. of ore concentrate: where the mixture was 50-50, about 12-15 lbs. of coal would be used, while for a 75 magnetite-25 hematite composite the coal content could be reduced to about 10 lbs./l.t.

The finely divided magnetite can be either natural or "artificial."

Illustrative of what can be accomplished with a different type of ore, a method for treating a Michigan Jasper ore will now be given.

### Example 3

The ore consisted (besides gangue material) mainly of specularite, and had an Fe content of about 36%. It was crushed to about 1 inch, and screened at three-eighths inch.

The amount of plus three-eighths material was approximately 40% by weight of the total. This coarse fraction was reductively roasted in a shaft furnace, converting substantially all of the specular hematite to magnetite. The roasted ore was then ground to minus 150 mesh, and was concentrated magnetically, giving a concentrate assaying 67% Fe and 4.8% Si and representing a weight recovery of 51%.

The minus three-eighths fraction (amounting to 60% by weight of the total) was ground to minus 65 mesh, 75

and was concentrated by anionic flotation. The flotation concentrate analyzed 63.3% Fe and 8.8% Si, and represented a weight recovery of 49%.

The two concentrates were filtered, and the filter cakes (moisture content about 8.0%) were thoroughly mixed, and to the mixture there were added 12 lbs./l.t. of bentonite and 20 lbs./l.t. of finely divided anthracite. These components were thoroughly mixed together, with the aid of a mixer-muller, and the homogeneous mixture was balled in a balling cone. The pellets, which were all minus 1 inch and plus one-fourth inch in diameter, were fed to the stockline of the same furnace as that described in Example 1, and at the same rate, and under the same conditions of temperature and rate of blowing.

15 The content of finely subdivided artificial magnetite made it possible to form green balls of satisfactory properties, and a fired ball satisfactory for transport and for steel plant use.

The fired balls when subjected to the A.S.T.M. standard 20 coke tumble test gave a hardness of 85.5 using a 10 mesh screen as the index figure.

In a companion run, in which the only condition 25 changed was that the magnetite concentrate was so finely ground that 95% of it consisted of particles finer than 325 mesh, the comparative strength data of the pellets averaged as follows:

|                                                                |       |
|----------------------------------------------------------------|-------|
| Drop test No. -----                                            | 7.5   |
| Compression test, green pellets ----- lbs. -----               | 13.4  |
| 30 Compression test, pellets dried at 250° F. ----- lbs. ----- | 42.0  |
| Compression test, pellets fired at 2450° F. ----- lbs. -----   | 1,280 |

These data illustrate the fact that a product of improved 35 quality can be made by insuring that a large part of the magnetite content is very finely ground, much finer than is needed for concentration purposes. In other words, smaller percentages of extremely fine grained magnetite can be made to serve essentially the same purposes as a larger percentage of a relatively coarser magnetite.

It should be mentioned, in connection with the above 40 specific examples, that the over-grinding of the artificial magnetite was for the purpose of providing sufficient ultra fines to give a network of grain growth-promoting crystals (of hematite derived from oxidizing the magnetite) for bonding the hematite particles. The same result 45 would have been realized had finely divided natural magnetite of the same particle size distribution been used in lieu of the artificial magnetite.

In repetitions of the process of the above specific examples it has been established that the magnetite addition 50 is useful not only in the case of hematite (earthy or specular) but also in the cases of hydrous iron oxide such as limonite, boggy ores and ores containing iron carbonate (siderite).

Hematite concentrates other than specularite concentrates 55 also frequently are difficult to ball and pelletize. This difficulty may come about not only because the mineral consists of hematite but also because of the coarseness of the concentrate and of a lack of fines due to the particular concentration process utilized. An example 60 of hematite material difficult to ball and pelletize by the usual procedures is a type of concentrate produced in the recovery of iron oxides from tailings currently produced or from tailings basins that have accumulated through the treatment of Mesabi Range iron ore.

In the recovery of iron values from a tailings basin in 65 the Western Mesabi District it was found that an acceptable recovery and grade of concentrate could be obtained by treating the tailings material by a combined process in which Humphrey spirals were used to recover the 70 coarser portion of the tailings and a flotation process was used to recover the fine mineral values. It was necessary to deslime the fine ore prior to flotation in order to make an effective separation. The composite concentrate of the spiral and flotation concentrate is shown in the middle column of Table II following:

TABLE II

| Mesh | Percent Weight                                     |                               |
|------|----------------------------------------------------|-------------------------------|
|      | Combined Spiral and Flotation Hematite Concentrate | Magnetic Taconite Concentrate |
| +20  | 0.5                                                | -----                         |
| +48  | 2.1                                                | -----                         |
| +65  | 10.5                                               | -----                         |
| +100 | 22.7                                               | -----                         |
| +150 | 20.3                                               | 1.1                           |
| +200 | 20.0                                               | 2.6                           |
| +325 | 16.4                                               | 8.7                           |
| +325 | 7.5                                                | 87.6                          |
|      | 100.0                                              | 100.0                         |

where it may be noted that the product had material in it as coarse as 20 mesh but had only 7.5% finer than 325 mesh. Because of the absence of fines it was impossible to ball or agglomerate this product.

However, it was found that if some finer ground magnetite concentrate were added to this product the resulting mixture could be both balled and agglomerated in a commercially acceptable manner. Tests were made in which a mixture of the spiral and flotation concentrate, assaying 58.5% iron and 7.5% silica, to the amount of 60% was mixed with 40% by weight of a magnetite concentrate made from taconite and ground to a size finer than usual, that this mixture could be satisfactorily balled and agglomerated. The analysis of the magnetite concentrate was 60.5% iron and 7.2% silica. Its sizing analysis is shown in Table II. The predominate minerals in the composite of spiral and flotation concentrates were earthy hematite and limonite. This 60-40 mixture was thoroughly mixed and filtered to give a filter cake containing 7.5% moisture, and to the filtered mixture were added 12 pounds of bentonite and 26 pounds of coal per long ton, dry weight, of the concentrate. The added magnetite gave sufficient plasticity to the admixture so that it was possible satisfactorily to ball this material in a standard balling drum. The resulting balls were then fired to a temperature of 2450° Fahrenheit in a shaft furnace of the type previously described and satisfactory pellets were made.

By the use of this technique it was possible to produce a satisfactory product from the spiral and flotation concentrate without regrinding it for the production of fines. The fired pellets product was also superior to fired pellets made from ground hematite alone, because of the network, around the hematite particles, of hematite which had been formed from the magnetite content during the heat-treatment, which network gave additional strength to the pelletized and indurated product.

On the Mesabi Range there are available tonnages of ore which have a desirable dry analysis but because of their high moisture content the natural iron content is low and they are therefore not economical to mine. Associated with such ores is material of a like nature but which has undesirable amounts of silica which must be removed to make the ore salable. Typical of such ores are those found in the Carmi Mine near Hibbing, Minnesota. Examples of typical ores from this property, one of which requires concentration and one needs only to be dried and agglomerated, are given below:

|              | Ore Analyses |                |                 |                   |                |           |
|--------------|--------------|----------------|-----------------|-------------------|----------------|-----------|
|              | Percent Iron | Percent Silica | Percent Alumina | Percent Ign. Loss | Percent Moist. | Nat. Iron |
| Ore "A"----- | 46.45        | 16.36          | 3.78            | 4.10              | 14.2           | 39.85     |
| Ore "B"----- | 57.65        | 7.61           | 4.58            | 4.22              | 17.8           | 47.38     |

These ores can be treated as follows:

Ore "A" which contains undesirable amounts of silica and which is quite sticky in nature is crushed to approximately  $\frac{1}{2}$ ", either by rolls or by hammer mill, and is then mixed with about 3% anthracite fines and then rolled, in a balling device of any conventional type, into small balls or pellets. Because of the sticky nature of the ore, the material balls readily even though some of the particles are as large as  $\frac{1}{2}$ ". These balls are then given a magnetic roast on a special type of horizontal traveling grate which is totally enclosed and through which reducing gases—either carbon monoxide or hydrogen or a mixture of the two—are caused to pass through the sinter bed. The temperature of the ore on the grate is held well below fusion temperatures, and under properly controlled conditions the primary iron minerals in the ore of hematite and limonite are converted almost entirely to the mineral magnetite. The balled product retains its original structure in the passage through the machine, and is cooled upon discharge in a reduced atmosphere below the temperature of re-oxidation. This roasted product is then wet ground to approximately 100 mesh, and concentrated by conventional types of low intensity magnetic separators. By so doing it is possible to obtain a magnetite concentrate that has a content of 59.15% iron, 7.52% silica and 3.2% alumina, and 1.05% ign. gain. I then take ore "B," which has an acceptable chemical analysis except for its moisture, and crush it to about  $\frac{1}{2}$ " as was done with ore "A." To this crushed product I add about 35% by weight of the fine ground magnetite concentrate made from ore "A." To this mixture of these two concentrates I add 12 pounds of bentonite and  $1\frac{1}{2}$  pounds of soda ash per long ton, dry weight, of the mixed ore and concentrate, and after admixing all ingredients I ball this material in a balling mechanism. Because of the sticky nature and high alumina content of ore "B" together with the fine concentrates from ore "A" this mixture balls exceptionally well. After balling the material is fired either in a shaft-type indurating furnace or on a traveling grate. The presence of the fine magnetite in the balls supplies heat to the indurating reaction and serves to act as a bond, holding together the particles of hematite. Moreover, the fine magnetite content of the ball is—during the induration procedure conducted in the presence of a hot gas mixture having a definitely oxidizing effect—converted to hematite and undergoes a definite grain growth, with the result that there is produced throughout the ball a network of bonding material between the (original) hematite particles bridging and cementing to neighboring grains through the medium of the ferric oxide produced by the oxidation of the fine magnetite which had been added prior to balling. This desirable result is illustrated in the accompanying drawing, in which Figures 1 and 2 are photolithographic reproductions of photomicrographs (taken at a magnification of 340) of typical cross-sections of indurated balls (or "pellets") produced in the experiment disclosed in specific Example 1 above. Figure 1 shows the coarse particles of specular hematite bonded together by finer hematite resulting from the oxidation of the magnetite content of the original mixture from which the ball had been formed. The bright white portions are relatively large particles of specular hematite, a typical particle being marked with the letter "H." The dark grey material, marked with the letter "L," is the "Lucite" mounting material used in preparing the cut-open pellet for polishing. A small particle of quartz is indicated at "Q," while the reference "M" leads to a relatively large particle of magnetite which had not—during the induration treatment—been completely converted to  $Fe_2O_3$ .

Figure 2, similarly marked, strikingly shows how the large specularite pieces are held together by a network bond of cemented-together finer particles of  $Fe_2O_3$  derived from the fine magnetite content of the original mix.

Both views indicate that the bond between the ore

particles occurs by bridging and cementation to neighboring grains through the medium of ferric oxide produced by the oxidation of the original content of added finely divided magnetite, which bridging, it is to be remembered, occurs in three dimensions. It is to be noted that there is substantially no indication, in either view, of any slag bonding: the bonding is through an intergrowth of hematite particles produced in situ amongst the larger specularite particles.

While the showing made in Figs. 1 and 2 pertains directly to Example 1, it equally applies to the other examples and is typical of the results flowing from the application of the principles of the present invention to the pelletization and induration of hematitic ore materials.

I claim:

1. In the agglomeration of a concentrate of a platy, granular non-magnetic iron ore containing less than 10% by weight of particles finer than 10 microns involving the step of forming a mixture of the concentrate and finely divided solid fuel into small balls by a rolling operation, the improvement which consists in homogeneously incorporating into said mixture finely divided magnetite in an amount by weight of from 15% to 75% of the total iron oxide of the resulting mixture, the particles of said finely divided magnetite being substantially all finer than 65 mesh and including from about 85% to about 94% of minus 200 particles.

2. In the agglomeration of a concentrate of granular hematite containing not more than a few percent of particles finer than 10 microns involving the step of forming a mixture of the hematite concentrate and finely divided solid carbonaceous fuel into small balls by a rolling operation, preliminary to a heat-treatment, the improvement which consists in homogeneously incorporating into said mixture a magnetite concentrate composed of particles most of which are of a size substantially smaller than are the hematite particles and which include a substantial proportion of particles finer than 10 microns, the amount of magnetite concentrate being from about 15% to about 75% by weight of the total iron oxide content of the resulting mixture.

3. The improved process defined in claim 2, characterized in that the magnetite concentrate is derived by reductively roasting a non-magnetic iron ore, finely grinding the roasted ore to an extent more than sufficient to

liberate the magnetite particles, and concentrating the finely ground ore.

4. Process of working up a concentrate of specular hematite ore into a form suitable for agglomeration, which consists essentially in homogeneously admixing with the specular hematite concentrate from about 20 to about 60 pounds, per long ton, of solid carbonaceous fuel and from 15% to 75% by weight of a magnetite concentrate composed of finely ground particles most of which are of a size materially smaller than are the specular hematite particles and which include a substantial proportion of particles finer than 10 microns, and balling up the homogeneous mixture by a rolling operation into pellets.
5. Process as defined in claim 4 in which the fineness of grind of the magnetite is in inverse ratio to the proportion of magnetite to specular hematite in the mixture.
6. Process of beneficiating a lean iron ore the iron content of which is mostly in the form of specularite, which comprises crushing and grinding the ore to the extent necessary for liberation of the specularite, separating from the ground ore a concentrate of specularite, adding to the specularite concentrate from about 20 to about 60 pounds, per long ton, of finely divided carbonaceous fuel, bentonite, and from 15% to 75% by weight of a magnetite concentrate composed of particles of a size substantially smaller than are the specularite particles and which include a substantial proportion of particles smaller than 10 microns, homogeneously admixing, balling up the homogeneous mixture into small balls by a rolling operation, and subjecting the small balls to induration treatment under conditions to effect oxidation and grain growth of the magnetite particles amongst the specularite particles.

- 35
- 30
- 35
- 40
- 45

#### References Cited in the file of this patent

#### UNITED STATES PATENTS

- 1,792,413 Christiansen ----- Feb. 10, 1931  
 2,743,172 De Vaney ----- Apr. 24, 1956

#### OTHER REFERENCES

- Mining Engineering (1), May 1950, pages 561-563.  
 Ban et al.: Mining Engineering (2), August 1953,  
 pages 803-811.